

# United States Patent

[11] 3,523,493

[72] Inventors Peter M. Berry  
Longueuil, Quebec, Canada;  
John Joe Kavalir, Two Mountains, Quebec,  
Canada  
[21] Appl. No. 657,230  
[22] Filed July 31, 1967  
[45] Patented Aug. 11, 1970  
[73] Assignee Uniroyal Inc.  
New York, New York  
a Corp. of New Jersey  
[32] Priority April 24, 1967  
[33] Canada  
[31] No. 988651

[56]

## References Cited

### UNITED STATES PATENTS

|           |         |                      |         |
|-----------|---------|----------------------|---------|
| 3,068,763 | 12/1962 | Harza .....          | 94/18   |
| 3,179,026 | 4/1965  | Crone .....          | 94/18   |
| 3,239,478 | 3/1966  | Harlan .....         | 260/27  |
| 3,265,765 | 8/1966  | Holden et al. ....   | 260/876 |
| 3,322,856 | 5/1967  | Holden et al. ....   | 260/876 |
| 3,325,430 | 6/1967  | Grasley .....        | 260/25  |
| 3,333,024 | 7/1967  | Haefele, et al. .... | 260/880 |
| 3,368,464 | 2/1968  | Thorp Jr .....       | 94/18   |

Primary Examiner— Jacob L. Nackenoff  
Attorney— Patrick Bright

[54] **COMPOSITION OF MATTER AND USE THEREOF  
IN JOINT SEALING**  
6 Claims, 2 Drawing Figs.

[52] U.S. Cl..... 94/18,  
260/876  
[51] Int. Cl..... E01c 11/10,  
C08f 15/00  
[50] Field of Search..... 260/876,  
2.3, 5; 94/18

**ABSTRACT:** There is disclosed a new composition of matter comprising a thermoplastic block copolymer of butadiene and styrene and reclaimed rubber and use thereof particularly for joint sealing purposes. This composition is extruded into a strip used to seal joints. In a preferred embodiment the extrusion is a hollow strip with flat sidewalls and slotted bottom, a special rubber cement as a primer is applied to the flat sidewalls of the strip and to the walls of the joint in the pavement or the like, whereupon the strip is inserted in the joint, the walls of the strip are allowed to spring outwardly into contact with the walls of the joint, and the solvent in the primer is then allowed to evaporate. Thus the uncured strip is cemented tightly in place.



Patented Aug. 11, 1970

3,523,493



INVENTORS.  
PETER M. BERRY  
JOHN J. KAVALIR  
BY  
Robert J. Patterson  
ATTORNEY

## COMPOSITION OF MATTER AND USE THEREOF IN JOINT SEALING

This invention relates to a new expansion joint composition, an expansion joint strip of novel design made therefrom, a method of sealing an expansion joint with such a strip and the resulting concrete paving assembly.

For many years strenuous efforts have been made to develop a satisfactory technique for sealing expansion joints in concrete highways, airport runways, and the like, in order to prevent the access of water and salt into the joint with resulting damage due to freezing of water and undesired chemical action of salt on the concrete in the joint area. So far as we are aware all previous proposals have been subject to various serious drawbacks.

It has recently been proposed to use a cured neoprene extrusion of complex multi-channel cross-section as an expansion joint sealant strip. According to this proposal, a cured extruded neoprene strip having narrow walls extending in criss-cross fashion from one side wall to the other side wall is inserted in the joint so as to be under compression. Typically the strip is compressed from 50 to 75% prior to its insertion. With this system there is very low adhesion of the strip to the walls of the joint. Because the strip is used only in compression and is not permanently adhered to the sides of the joint, relative up and down movement of the adjoining concrete slabs as traffic passes over the joints gradually causes the strips to work loose so that they project above the pavement and soon are pushed out altogether. The loose strips are a serious traffic hazard. This propensity of the strips to come out of the joints has ruled out altogether the use of this system on airport runways because of the danger that the strips will be sucked into jet engines. Also the strips are expensive and difficult to apply.

Our invention involves a novel approach to the expansion joint problem. In our system the walls of an uncured strip are permanently bonded to the walls of the joint so that the joint is completely sealed against access of water, salt, etc. The strip is so designed that in combination with this permanent bonding feature it can expand or contract freely with the contraction and expansion of the concrete slabs without reducing or interfering with the integrity of the seal. The permanent strong bonding feature is made possible by making the strip from a special uncured composition which we have invented and which is fully described below.

In the accompanying drawing, FIG. 1 is a cross-section of an expansion joint strip made according to our invention, prior to its insertion in the joint, and FIG. 2 is a cross-section of the finished joint assembly.

In practicing our invention we first prepare a mixture of (1) a thermoplastic polymer selected from the group consisting of a block copolymer having the general configuration A-B-A wherein the A's are polymeric blocks of alkenyl aromatic hydrocarbons typified by styrene, each A having an average molecular weight of 2,500 to 100,000 and B is a polymeric block of a conjugated diene, typified by butadiene, having an average molecular weight of 25,000 to 500,000 and hydrogenated derivatives of such block copolymers and (2) reclaimed rubber. The block copolymer, whether hydrogenated or not, is fully described in Canadian Patent 740,027 which is hereby incorporated herein by reference. Any kind of reclaimed rubber may be used, examples being neoprene reclaim, SBR reclaim including high styrene SBR (made with an unusually high styrene-butadiene ratio or by blending regular SBR with a high styrene-low butadiene resinous copolymer) reclaim, butyl reclaim, natural rubber reclaim, butadiene-acrylonitrile rubber reclaim, EPDM reclaim, etc. Instead of using a single kind of reclaim we can use a plurality of types of reclaim.

The reclaimed rubber component of our composition is the rubber compounding material commonly and widely available under the designation "reclaimed rubber" or "rubber reclaim" and as is well-known made by reclaiming vulcanized natural or synthetic rubber, especially that in scrap form, by methods which are equally well-known to the art. Examples of

the many descriptions of this widely known and commonly used material are those found in the following recognized authorities:

"Introduction to Rubber Technology", edited by Morton, published by Reinhold, 1959.

"Reclaimed Rubber" by Ball, published by Rubber Reclaimers Association, Inc., New York, 1947.

"Synthetic Rubber", edited by Whitby, published by Wiley, 1954, Chapter 17.

10 India Rubber World, articles on pages 772-774 of September, 1953 issue and pages 63-67 of October, 1953 issue.

The relative proportions of the block copolymer and reclaimed rubber can be varied widely depending upon the properties, including physical properties, desired in the joint sealing material. Preferably we use from 50 to 200 parts by weight of rubber reclaim per 100 parts of block copolymer.

15 In order to facilitate extrusion of the block copolymer-reclaim composition into the desired strip and to confer on the strip the desired physical properties, particularly at low temperatures which may be as low as -40°F., we prefer to incorporate substantial proportions of an extrusion aid or aids and one or more compatible plasticizers, typically employing from 5 to 45 parts of extrusion aid and 25 to 100 parts of plasticizer with 100 parts of the block copolymer and from 50 to 200 parts of rubber reclaim, all parts being by weight.

20 The preferred extrusion aid is mineral rubber which, as is well-known in the art, is a bituminous material, typified by gilsonite or blown petroleum asphalt and described for example on pages 749 and 750 of "The Chemistry and Technology of Rubber" by Davis and Blake, (published 1937 by Reinhold) and on page 157 of "Modern Rubber Chemistry" (published 1948 by Van Nostrand) by Barron.

25 Other extruding aids known to the art may be used in place of or in addition to mineral rubber. One such extruding aid which gives excellent results when used in relatively small amounts in conjunction with mineral rubber, is a fatty acid soap.

30 As the plasticizer component we may use any non-volatile plasticizer or plasticizers compatible with the other components of the mixture and typified by monomeric esters such as tricresyl phosphate, dioctyl phthalate, etc., plasticizing resins for example a plasticizing resin derived from urea-formaldehyde and exemplified by "Plastigen G" made by BASF, a plasticizing polyester or alkyd resin, often termed a polymeric ester plasticizer, exemplified by the resinous polyester materials sold under the trademark "Paraplex" made by Rohm & Haas, etc., or non-volatile petroleum oils commonly used as extender oils for rubbery materials, exemplified by "Circosol 4240/42 x H" and "Circolight" oils both made by Sun Oil Co. As already indicated, we may use several plasticizers instead of only one.

35 For certain installations, where black expansion joint seals are not desired, we may make light-colored or even pastel-colored strips by appropriate selection of the components. The most important factors in determining the color of the extruded strip are the colors of the reclaim, extrusion aid and plasticizers. If desired, pigments other than the pigment supplied by the reclaim can be included for particular color effects, for example where expansion joints in colored concrete are to be filled.

40 The several components of the composition of our invention are intimately mixed together in any suitable way well-known in the rubber art, to achieve a good mixture. This mixture is then extruded in the conventional manner used in rubber technology using an extrusion die shaped to give the desired cross-section portrayed in the drawing. The extruded strip is now ready for installation. For installation it may be supplied in reels from which it can simply and rapidly be fed into the joint, using suitable applicator equipment for applying the primer described below to the walls of the joint and to the strip.

45 By proceeding as described above, we obtain a strip having nearly ideal physical properties for expansion joint purposes. Typically the elongation of the material of our strip ranges

from 500 to 1000% over a temperature range of from -40°F. to +120°F.; this range embraces the temperatures commonly encountered in this country. Its resiliency and hardness are such as to prevent the undesired penetration of stones, gravel, etc. into the joint, which would destroy its effectiveness, and yet the hardness is not so great at sub-zero temperatures such as 40°F. as to make the strip brittle. With regard to elasticity, the material returns, after elongation to 200%, almost immediately to its original length and after elongation to 1000% returns to 150% of its original length within 1 minute and to its original length within 5 minutes.

Referring to FIG. 1, the extruded strip comprises downwardly and outwardly extending side walls 2, a trough-like upper wall constituting a hinge formed by portions 3 which slope downwardly and merge at the center 4 in such a way that when the strip 1 is compressed laterally for insertion it will not bulge upwardly, and integral downwardly and inwardly extending projections 5 which terminate short of the center so as to allow compression of the strip just prior to insertion in the joint. These projecting portions 5 are pointed as indicated at 6 to facilitate insertion. The outer walls 7 of projections 5 are sloped so that the projections together have a pointed configuration which facilitates such insertion.

The design of strip 1 as extruded is such that when the depending side members formed by side walls 2 and projections 5 are pushed towards one another to the point where the outer faces 8 of walls 2 are substantially parallel to each other, the distance between faces 8 is only very slightly wider than the width of the joint to be filled. Thus the extrusion is predesigned to fit a joint of a particular width. The design of the extrusion 1 portrayed in FIG. 1 is such that there is a hinging action of the depending side members. In other words, portions 3 constitute a hinge and the characteristics of the material from which the extrusion is made are inherently such that when the depending portions are pushed inwardly towards one another and then released they resume, so far as they can, the original position they had in the extrusion as it was formed. These features are extremely important in achieving the results of our invention.

Now referring particularly to FIG. 2, in sealing a joint in accordance with our invention, we first coat the upper portion of the walls 9 of the adjacent concrete slabs 10 with a layer 11 of a primer which is a neoprene cement (i.e. an organic solvent solution of neoprene containing a curative or curatives) capable of forming in cooperation with the material of the extrusion an adhesive bond which permanently and strongly bonds the walls 2 of the strip 1 to the concrete and forming a fluid-tight seal therebetween. This primer also penetrates the permeable walls of the concrete slabs thereby strengthening the concrete and, more importantly, preventing accidental in-

filtration of water or salt solution into the concrete next to the joint and into the joint area itself. The faces 8 of strip 1 are also coated with this primer cement just prior to insertion of the strip. The strip is then inserted into the joint and properly positioned as by means of a profiled roller. The solvent from the primer immediately starts to dissolve the material constituting the strip. After insertion the strip expands so as to position its side walls against the concrete. Rapid evaporation of the organic solvents in the primer takes place through the pores of the adjoining concrete. The result is that within 1/2 to 1 hour, depending on atmospheric conditions and the solvents used, a perfect physical bond between the walls of the strip and the concrete is achieved and the pavement can be opened to traffic. Because of curing of the neoprene in the primer, which starts immediately upon evaporation of the organic solvents, maximum adhesion between strip and concrete is obtained within 2 to 3 days after insertion.

While our invention is usually applied to expansion joints formed between slabs of concrete it can also be applied in exactly the same way already described to expansion joints formed between a concrete slab and a rigid steel member or between two rigid steel members, such as are often encountered in bridges.

A typical primer formulation suitable for use in our invention is a so-called "rubber cement" made from neoprene compounded with suitable curatives, such as magnesium oxide or zinc oxide or both, an antioxidant if desired and a phenolic resin or resins of the type commonly used in making neoprene cements, all dissolved and suspended in a suitable volatile organic solvent or solvents also of known type to give an appropriate total solids content. One such formulation which we have found to give outstanding results is as follows:

|                                                                                                                                                                            |     | Parts by weight |
|----------------------------------------------------------------------------------------------------------------------------------------------------------------------------|-----|-----------------|
| Neoprene AF (so-called self-curing neoprene).....                                                                                                                          | 100 |                 |
| Magnesium oxide (curative for neoprene).....                                                                                                                               | 4   |                 |
| Zinc oxide (curative for neoprene).....                                                                                                                                    | 5   |                 |
| Antioxidant.....                                                                                                                                                           | 1   |                 |
| Heat-reactive oil-soluble tertiary butyl phenol-formaldehyde resin (such as "TR-14634" made by Union Carbide).....                                                         | 45  |                 |
| Thermoplastic Terpene-modified phenol formaldehyde resin, typically having a capillary melting point of about 335° F. (such as "Durez 12603" made by Hooker Chemical)..... | 50  |                 |
| Ethyl acetate.....                                                                                                                                                         | 60  |                 |
| Toluol.....                                                                                                                                                                | (1) |                 |

<sup>1</sup> To a total solids content of 22%.

#### EXAMPLES 1 TO 7

The specific examples given in the table illustrate our invention. All parts are by weight.

|                                     | Example |        |        |        |        |        |        |
|-------------------------------------|---------|--------|--------|--------|--------|--------|--------|
|                                     | 1       | 2      | 3      | 4      | 5      | 6      | 7      |
| "Kraton 101" <sup>1</sup> .....     | 100.00  | 100.00 | 100.00 | 100.00 | 100.00 | 100.00 | 100.00 |
| Neoprene reclaim.....               | 160.00  |        |        |        |        |        | 75.00  |
| SB R reclaim.....                   |         | 150.00 |        |        |        |        |        |
| Butyl reclaim.....                  |         |        | 150.00 |        |        |        |        |
| High-styrene SB R reclaim.....      |         |        |        | 150.00 |        |        |        |
| High-styrene SB R reclaim.....      |         |        |        |        | 150.00 |        |        |
| Natural rubber reclaim.....         |         |        |        |        |        | 150.00 |        |
| Mineral rubber <sup>2</sup> .....   | 10.00   | 10.00  | 10.00  | 10.00  | 10.00  | 10.00  | 10.00  |
| Triresyl phosphate.....             | 15.00   | 15.00  | 15.00  | 15.00  | 15.00  | 15.00  | 15.00  |
| "Plastigen G-50" <sup>3</sup> ..... | 10.00   | 15.00  | 15.00  | 15.00  | 15.00  | 10.00  | 10.00  |
| "Nu-Slip" (Fatty acid soap).....    | 2.00    | 2.00   | 2.00   | 2.00   | 2.00   | 2.00   | 2.00   |

#### Typical Physical Properties at R.T. (76° F.)

|                          |       |       |       |       |       |       |       |
|--------------------------|-------|-------|-------|-------|-------|-------|-------|
| Tensile.....             | 1,280 | 1,855 | 1,240 | 1,140 | 1,480 | 1,285 | 1,210 |
| Elongation, percent..... | 865   | 945   | 835   | 790   | 840   | 880   | 850   |
| Modulus:                 |       |       |       |       |       |       |       |
| 100%.....                | 210   | 220   | 190   | 220   | 215   | 150   | 110   |
| 200%.....                | 255   | 285   | 245   | 265   | 285   | 180   | 130   |
| 300%.....                | 295   | 355   | 305   | 315   | 335   | 240   | 160   |
| Shore "A" hardness.....  | 57    | 55    | 64    | 55    | 56    | 54    | 57    |

<sup>1</sup> A styrene-butadiene block copolymer of the type shown in Canadian Patent 740,027.

<sup>2</sup> Blown petroleum asphalt, Melting Pt. 300-315° F.

<sup>3</sup> Plasticizing resin of medium viscosity derived from urea-formaldehyde condensation product.

It will be understood that the views of the drawing are greatly enlarged since the width of expansion joints generally ranges from 1/4 inch to 1 inch.

From the foregoing description it will be seen that we have invented a novel system for sealing expansion joints in concrete pavement, which system is perfectly adapted for use in highways, airport runways and the like and gives many advantages over previously proposed systems. The several features of our invention cooperate in a new way to achieve these new results. The essential features which provide these results are the composition of the expansion joint material itself, the design of the extrusion and the primer system. The fact that the joint material is uncured is a key factor in our system because it enables the requisite permanently strong adhesive bond between it and the walls of the joint to be achieved. If a cured material were used for the strip it would not be possible to develop the requisite permanently strong adhesive bond which is at the heart of our invention. Another important feature of our invention is that the extrusion strip material is resilient so that after being laterally compressed for insertion into the joint and then released the depending side portions of the strip immediately spring outwardly and contact the joint walls with sufficient force to hold the strip in place until the strong adhesive bond is established.

It will be understood that this description of our invention is illustrative and that numerous modifications thereof can be made without departing from the spirit of our invention.

#### OTHER USES OF OUR COMPOSITION

Our composition of matter is adapted to many other uses than for sealing expansion joints in pavements, bridges, runways, etc. Thus we can use our expansion joint technique for sealing expansion joints generally, for example the vertical expansion joints in so-called parapets which are vertical walls at the edges of highways and the like. We can also use our composition, typically in the form of an extrusion of suitable cross section, anywhere in construction where it is desired to seal against the entrance of water or outside air or against the leakage of water or air. Thus, we can use it for sealing against the leakage of hot or cold conditioned air from the interior of a building to the atmosphere. We can use our technique in so-called curtain wall building construction for sealing the joints between adjacent exterior vertical wall panels. We can use it for sealing the joints around doorways, windows, etc. In certain wall applications, we generally prefer to use an extrusion much like that shown in FIG. 1 except that the outer (i.e., upper as viewed in that figure) face is completely flat, instead of trough-like, in order that when the extrusion is installed in the joint the outer face of the extrusion will be flush with the panels and give a pleasing appearance. The color of the extrusion and the primer used to bond it in place will of course be adjusted so as to match the color of the surrounding structure.

Our composition can also be used for sealing the joints between doors, windows and other elements of a building and the structure of the building proper. Thus, it can be used, preferably in the form of a triangular extrusion, for corner joints such as are encountered around the frames of doors and windows, the primer being applied over the area which must be sealed in order to hold the extrusion in position. It can also be used for sealing glass in a window frame; in this application it may be extruded in the form of a channel which is slipped over the edges of the glass prior to positioning in the frame, the glass being subsequently locked in place in any obvious way. Our composition can also be used as a weather stripping material; in this usage the composition is typically applied as an extrusion of varying design such that one side is adhered to a rigid member and another portion of the extrusion is hinge-like and is compressed by the closing of the door or window in order to provide the necessary seal.

Our composition is also well adapted to be used in sheet form, typically calendered, for flashing and roofing. For flashing or roofing applications we apply a suitable organic solvent, such as for example toluol or xylol, which can be used either

by itself or in the form of a rubber cement, to the roofing substructure in order to effect permanent bonding of the flashing or roofing. In roofing applications we typically place large sheets of our composition in position with slight overlapping at the edges and we effect fusion of the material in the overlapping area to form an integral joint by the application of an organic solvent or rubber cement of the type just referred to; such fusion of the material in the overlapping areas is possible because our composition is uncured.

- 10 Our composition can also be used in sheet form for holding water in irrigation ditches or basins or in the reservoirs behind dams. In this application large sheets of the material are disposed in slightly overlapping fashion over the earth area and the overlapping portions of the sheets are fused in the manner just described. In this application for greater strength and tear resistance we often prefer to admix reinforcing fibrous material with our composition at the time of its preparation. Any suitable fibrous material may be employed for this purpose, examples being sisal, cotton fiber, nylon fiber, ground uncured rubberized textile fabric cuttings which are formed as waste in the manufacture of pneumatic tires, etc.

Accordingly it will be seen that the composition of our invention has a great many useful applications. It will be understood of course that the foregoing is by no means a complete enumeration of the uses to which our composition may be put.

We claim:

- 30 1. A composition of matter comprising the following components:

(1) a polymer of the group consisting of a block copolymer having the general configuration A-B-A wherein the A's are polymeric blocks of alkenyl aromatic hydrocarbons, each A having an average molecular weight of 2,500 to 100,000 and B is a polymeric block of a conjugated diene having an average molecular weight of 25,000 to 500,000 and hydrogenated derivatives thereof,

(2) reclaimed rubber made by devulcanizing cured diene rubbers,

(3) an extrusion aid selected from the group consisting of mineral rubber, fatty acid soap, and mixtures thereof, and

(4) plasticizer selected from the group consisting of monomeric esters, plasticizing resins, non-volatile rubber extender oils, and mixtures thereof in relative proportions by weight of from 50 to 200 parts of reclaimed rubber, from 5 to 45 parts of extrusion aid, and from 25 to 100 parts of plasticizer per 100 parts of said polymer.

2. A joint sealing strip comprising an uncured extrusion of a composition of matter comprising the following components:

(1) a polymer of the group consisting of a block copolymer having the general configuration A-B-A wherein the A's are polymeric blocks of alkenyl aromatic hydrocarbons, each A having an average molecular weight of 2,500 to 100,000 and B is a polymeric block of a conjugated diene having an average molecular weight of 25,000 to 500,000 and hydrogenated derivatives thereof, and

(2) reclaimed rubber made by devulcanizing cured diene rubbers, in relative proportions by weight of from 50 to 200 parts of reclaimed rubber per 100 parts of said polymer.

3. A joint sealing strip comprising an uncured extrusion of a composition of matter comprising the following components:

(1) a polymer of the group consisting of a block copolymer having the general configuration A-B-A wherein the A's are polymeric blocks of alkenyl aromatic hydrocarbons, each A having an average molecular weight of 2,500 to 100,000 and B is a polymeric block of a conjugated diene having an average molecular weight of 25,000 to 500,000 and hydrogenated derivatives thereof,

- (2) reclaimed rubber made by devulcanizing cured diene rubbers,
  - (3) an extrusion aid selected from the group consisting of mineral rubber, fatty acid soap, and mixtures thereof, and
  - (4) plasticizer selected from the group consisting of monomeric esters, plasticizing resins, non-volatile rubber extender oils and mixtures thereof in relative proportions by weight of from 50 to 200 parts of reclaimed rubber, from 5 to 45 parts of extrusion aid, 10 and from 25 to 100 parts of plasticizer per 100 parts of said polymer.
4. An expansion joint sealing strip comprising an uncured extrusion of a composition comprising
- (1) a polymer of the group consisting of a block copolymer having the general configuration A-B-A wherein the A's are polymer blocks of alkenyl aromatic hydrocarbons, each A having an average molecular weight of 2,500 to 100,000 and B is a polymeric block of a conjugated diene having an average molecular weight of 25,000 to 500,000 and hydrogenated derivatives thereof, and
  - (2) reclaimed rubber made by devulcanizing cured diene rubbers in relative proportions by weight of from 50 to 200 parts of reclaimed rubber per 100 parts of said polymer, said extrusion having downwardly and outwardly extending side walls, an integral trough-like upper wall and having its lower portion formed by integral downwardly and inwardly extending pointed projections terminating short of the center.
5. The method of sealing an expansion joint in a concrete pavement which comprises coating the adjacent walls of the concrete slabs forming the joint with a primer comprising a neoprene cement, placing in the joint an uncured extrusion of a composition comprising the following components:
- (1) a polymer of the group consisting of a block copolymer having the general configuration A-B-A wherein the A's are polymeric blocks of alkenyl aromatic hydrocarbons, each A having an average molecular weight of 2,500 to 100,000 and B is a polymeric block of conjugated diene having an average molecular

- weight of 25,000 to 500,000 and hydrogenated derivatives thereof, and
- (2) reclaimed rubber made by devulcanizing cured diene rubbers in relative proportions by weight of from 50 to 200 parts of reclaimed rubber per 100 parts of said polymers, said extrusion prior to placement having downwardly and outwardly extending side walls, an integral trough-like upper wall, and having its lower portion formed by integral downwardly and inwardly extending pointed projections terminating short of the center, said extrusion prior to placement being slightly wider than the joint and having its side walls coated with said primer, allowing said strip to expand outwardly in the joint so that said side walls press against the primed walls of the concrete slabs in parallel relationship to said primed walls with said projections terminating short of the center of the joint, and allowing the solvent in the primer to diffuse and the primer to set and permanently and strongly bond said side walls to the walls of the joint.
6. A concrete pavement comprising adjacent concrete slabs having spaced walls forming an expansion joint, and disposed in said joint an uncured extrusion of a composition comprising the following components:
- (1) a polymer of the group consisting of a block copolymer having the general configuration A-B-A wherein the A's are polymeric blocks of alkenyl aromatic hydrocarbons, each A having an average molecular weight of 2,500 to 100,000 and B is a polymeric block of a conjugated diene having an average molecular weight of 25,000 to 500,000 and hydrogenated derivatives thereof, and
  - (2) reclaimed rubber made by devulcanizing cured diene rubbers in relative proportions by weight of from 50 to 200 parts per 100 parts of said polymer, said extrusion having a trough-like upper wall, integral parallel side walls permanently and strongly bonded to the walls of the joint by a primer and having its lower portions formed by integral downwardly and inwardly extending pointed projections terminating short of the center.